

# United States Patent Office

2,913,414

Patented Nov. 17, 1959

1

2,913,414

## PETROLEUM LUBRICANTS STABILIZED AGAINST HYDROCARBON METABOLIZABLE MICROORGANISMS

Edward B. Hodge, Terre Haute, Ind., assignor to Commercial Solvents Corporation, Terre Haute, Ind., a corporation of Maryland

No Drawing. Application August 1, 1957  
Serial No. 675,529

3 Claims. (Cl. 252—51.5)

My invention relates to a stabilized petroleum lubricant and more particularly to a process for the production of stabilized petroleum lubricants containing as the active stabilizing agent compounds having the following structural formula:



where X is selected from the group consisting of hydrogen and bromine, R is selected from the group consisting of methyl and ethyl and R' is selected from the group consisting of aryl, substituted aryl and heterocyclic.

It is well known that organisms from the group consisting of *Corynebacterium*, *Achromobacter*, *Nocardia*, *Pseudomonas* and *Mycobacterium* metabolize petroleum hydrocarbons and fatty acids and thereby produce undesirable oxidation products.

The petroleum industry has long been interested in the stabilization of various petroleum products such as cutting oils, hydraulic fluids, etc. against break-down by bacteria which metabolize the hydrocarbons with the concurrent formation of deleterious metabolites.

Many compounds have been used as stabilization agents in lubricants, but very few have been found to be commercially successful due to the fact that the compounds are unstable, or are not active against a wide variety of microorganisms.

Among the active compounds which are useful in my invention are 2-nitro-2-bromo-1-methoxy-1-phenylbutane, 2-bromo-1-p-chlorophenyl-1-methoxy-2-nitropropane, 2-bromo-1-ethoxy-2-nitro-1-phenylpropane, 2-bromo-1-methoxy-1-p-methoxyphenyl-2-nitrobutane, 1-(2-furyl)-2-bromo-1-methoxy-2-nitropropane, 1-(2,4-dichlorophenyl)-1-methoxy-2-nitrobutane, 1-(2-pyridyl)-2-bromo-1-methoxy-2-nitropropane, etc. Of these compounds, I prefer to utilize 2-nitro-2-bromo-1-methoxy-1-phenylpropane as it is very active against petroleum metabolizing bacteria, while being relatively inexpensive. These compounds can be easily prepared in good yields by the method set out in U.S. Patent 2,742,395.

I have found that in some instances I can obtain total inhibition of bacterial growth in petroleum lubricants at concentrations as low as 0.005%. I prefer to include at least 0.0075% in most petroleum formulations. However, I can employ amounts up to 10.0% of the active agent when the latter is soluble to this extent in the particular petroleum hydrocarbon compositions.

The active ingredients of my invention are effective bacteriostatic agents in petroleum containing lubricants such as cutting oils, penetrating oils, grinding lubricants, iron tinning lubricants, core oils, hydraulic fluids, etc.

The following examples set out lubricating compositions in which my active ingredients are effective bacteriostatic agents. It is not intended that my invention be limited to the compositions, portions, or lubricants set out below, but rather I intend for all the equivalents

2

and variations obvious to those skilled in the art to be included within the scope of this specification and the attached claims.

### Example I

5 A water-soluble cutting oil containing 2-nitro-2-bromo-1-methoxy-1-phenylpropane was tested for activity against petroleum metabolizing organisms by preparing a cutting oil composition having the formula:

|                             | Percent by weight |
|-----------------------------|-------------------|
| Light mineral oil           | 85                |
| Oleic acid                  | 10                |
| 2-amino-2-methyl-1-propanol | 5                 |

10 15 Two equal portions of this formulation were prepared and enough 2-nitro-2-bromo-1-methoxy-1-phenylpropane to create a 750  $\gamma$ /ml. concentration was added to one portion. Both portions were then diluted 1:10 with North Gelatin Agar (Difco) and streaked with an 18 hour agar slant culture of the representative organism *Pseudomonas aeruginosa*. The control and the stabilized composition were then incubated for 18 hours at 35° C. and the growth recorded. No growth was exhibited on the stabilized composition while a growth of 4+ was noted on the control composition.

### Example II

A steam cylinder oil having the following composition:

|    |                                           |              |     |
|----|-------------------------------------------|--------------|-----|
| 30 | S.A.E. lubricating oil                    | percent      | 90  |
|    | Oleic acid                                | do           | 10  |
|    | 2-nitro-2-bromo-1-propoxy-1-phenylpropane | $\gamma$ /ml | 750 |

35 35 was diluted and tested as shown in Example I. The stabilized composition was found to exhibit no bacterial growth while the control composition exhibited a growth of 4+.

### Example III

40 A core oil having the following composition:

|                                                        |              |      |
|--------------------------------------------------------|--------------|------|
| Crude tall oil                                         | percent      | 25   |
| Fuel oil                                               | do           | 35   |
| Tall oil ester (glycol or glycerol)                    | do           | 40   |
| 2-bromo-1-(3,4-dichlorophenyl)-1-methoxy-2-nitrobutane | $\gamma$ /ml | 1000 |

50 55 was diluted and tested as shown in Example I and found to exhibit no bacterial growth while the control composition exhibited a growth of 4+.

### Example IV

A cutting oil and grinding lubricant having the following composition:

|                                              |              |     |
|----------------------------------------------|--------------|-----|
| Tallow                                       | percent      | 65  |
| Paraffin wax                                 | do           | 29  |
| Bees wax                                     | do           | 1   |
| Citric acid                                  | do           | 1.3 |
| 60 Oxalic acid                               | do           | 1.3 |
| Potassium citrate                            | do           | 1.3 |
| Urea                                         | do           | 0.4 |
| 1-(2-furyl)-2-bromo-1-methoxy-2-nitropropane | $\gamma$ /ml | 750 |

65 65 was diluted and tested by the method of Example I and found to exhibit no bacterial growth while a control composition exhibited a growth of 4+.

70 Now having described my invention, what I claim is:

1. A petroleum hydrocarbon oil of lubricating viscosity stabilized against hydrocarbon metabolizable microorganisms containing in a small but sufficient amount to inhibit

bacterial growth in said petroleum lubricant a compound having the following structural formula



5

where X is selected from the group consisting of hydrogen and bromine, R is selected from the group consisting of methyl and ethyl and R' is selected from the group consisting of aryl, chloro and methoxy substituted aryl and heterocyclic.

2. An aliphatic petroleum hydrocarbon oil of lubricating viscosity stabilized against hydrocarbon metabolizable microorganisms containing from 0.005% to 10.0% by weight of a compound having the structural formula:



where X is selected from the group consisting of hydrogen and bromine, R is selected from the group consisting of methyl and ethyl and R' is selected from the group consisting of aryl, chloro and methoxy substituted aryl and heterocyclic.

10

3. An aliphatic petroleum hydrocarbon oil of lubricating viscosity stabilized against hydrocarbon metabolizable microorganisms containing 0.0075 to 10.0% of a compound having the structural formula:



where X is selected from the group consisting of hydrogen and bromine, R is selected from the group consisting of methyl and ethyl and R' is selected from the group consisting of aryl, chloro and methoxy substituted aryl and heterocyclic.

15

#### References Cited in the file of this patent

#### UNITED STATES PATENTS

|           |              |       |               |
|-----------|--------------|-------|---------------|
| 2,562,151 | Senkus       | ----- | July 24, 1951 |
| 2,742,395 | Hodge et al. | ----- | Apr. 17, 1956 |
| 2,780,598 | Cafcas       | ----- | Feb. 5, 1957  |

#### OTHER REFERENCES

"Fundamentals of Microbiology," by Frobisher, 5th ed., 1953, W. B. Saunders Co., p. 3.